

## UNITED STATES PATENT OFFICE

2,478,420

STEEL FOR PLASTIC MOLD DIES AND  
ARTICLES MADE THEREFROM

Peter Payson, New York, N. Y., assignor to Crucible Steel Company of America, New York, N. Y., a corporation of New Jersey

No Drawing. Application March 13, 1947,  
Serial No. 734,554

5 Claims. (Cl. 75—128)

## 1

This invention pertains to mold dies for the compression-molding of resinous plastics, and to a low carbon, low alloy chrome-manganese-molybdenum steel, which may also contain small amounts of either or both nickel and boron, and which is especially suited for use in mold dies of the character aforesaid.

Mold dies for the compression-molding of thermosetting synthetic resin powders, such as the phenol-, urea- or melamine-aldehyde resins, are made by hubbing, i. e., by pressing, into a relatively soft steel block, an impression of the resinous object to be molded therefrom. The hubbing is effected by means of a hard steel die which has been machined or engraved to the shape and configuration of the object to be molded, and which is impressed under tremendous hydraulic pressure into the aforesaid relatively soft steel die block. After the hubbing operation is completed, the resulting impression-containing die block is carburized, and then heat treated by a conventional quench and temper treatment.

The principal requirements of a suitable steel for plastic mold dies, are that (1) it must be easy to hub; (2) it must be susceptible to carburization; (3) it must have good hardenability so that after it is carburized, the die can be hardened by an oil quench, rather than a water quench in order that the case or carburized part of the die will have high hardness and the core, or uncarburized part of the die, will have fair strength to support the case of the die under the rather heavy pressures of about one to four tons per square inch employed in the compression molding of resinous plastics; and (4) it must be inexpensive. Typical analyses of the steels most commonly used for this purpose hitherto are as follows:

Table I

| Grade | C   | Mn  | Si  | Ni   | Cr   | Bal. |
|-------|-----|-----|-----|------|------|------|
| A     | .05 | .15 | .10 |      |      | Fe   |
| B     | .07 | .50 | .20 | 1.25 | .65  | Fe   |
| C     | .10 | .50 | .20 | 3.50 | 1.60 | Fe   |

## 2

Steel A can be annealed to a very low hardness and is easy to cold hub, but it has very poor hardenability and dies made from it have to be quenched in water with accompanying risk of distortion in order to be hardened satisfactorily and even with a water quench the attainable hardness at the core of the die is quite low. Steel B has fairly good hardenability and dies made from it therefore, can be quenched in oil after they are carburized and attain high hardness at the surface and fair hardness at the core, but this steel is definitely inferior to steel A in hubbability. Steel C has excellent hardenability but even when it is fully annealed it is too hard for efficient cold hubbing, and dies made from it have to be machine cut which is much more expensive than cold hubbing.

I have discovered an analysis of steel which is applicable for plastic mold dies, which can be cold hubbed almost as easily as steel A, and which has hardenability much better than that of steel A and at least equal to that of steel B. I have balanced the composition of this steel so that it contains in suitable proportions the elements Mn, Ni, Cr, and Mo which appreciably improve the hardenability of the steel but which at the same time do not appreciably lower the hubbability of the steel. The elements least effective in increasing the hardness of ferrite, and therefore the hardness of the fully annealed steel, which controls the hubbability of the steel, are Cr, Ni, Mo, Mn, and Si, in the order named. The elements most effective in increasing the hardenability of steel are Mn, Mo, Cr, Si, and Ni, in the order named. Therefore, for optimum results in a steel for plastic mold dies I select the elements near the top of each list. I use an appreciable amount of Cr because it has least effect on hubbability and an appreciable effect on hardenability. I use a small amount of Si, just sufficient to assure adequate deoxidation of the steel, because this element has the most deleterious effect on hubbability and little effect on hardenability. I use intermediate amounts of Mn and Ni because although Mn has a great effect on hardenability it also seriously affects hubbability whereas al-

though Ni has a relatively minor effect on hardenability, it also has a relatively minor effect on hubbability. I use a relatively small amount of Mo because although it has a great effect on hardenability and a relatively small effect on hubbability, it is the most expensive of the elements in this steel. Finally I may use a very small amount of boron which has a relatively small effect on hubbability and an appreciable effect on hardenability. High carbon has a serious effect on hubbability and therefore it is kept as low as feasible, generally under 0.10%.

The broad range for my improved steel for plastics mold dies is:

5

Table III

| Steel | Designation               | Hardness Brinell |
|-------|---------------------------|------------------|
| D     | Plain carbon (per A)..... | 89               |
| F     | This invention.....       | 99               |
| G     | do.....                   | 99               |
| K     | do.....                   | 99               |
| H     | do.....                   | 103              |
| J     | do.....                   | 107              |
| E     | Lower Ni-Cr (per B).....  | 109              |
| L     | Higher Ni-Cr (per C)..... | 137              |

Further tests on hubbability were made by measuring the diameter of the impression made in

| Percent C | Percent Mn | Percent Si | Percent Ni | Percent Cr | Percent Mo | Percent B   |
|-----------|------------|------------|------------|------------|------------|-------------|
| .02/.15   | .10/1.00   | .00/.40    | .00/1.00   | .80/3.00   | .10/1.00   | .0000/.0050 |

The preferred analysis is:

the different steels with a 10 mm. ball under a load

| Percent C | Percent Mn | Percent Si | Percent Ni | Percent Cr | Percent Mo | Percent B |
|-----------|------------|------------|------------|------------|------------|-----------|
| .02/.07   | .30/.50    | .02/.20    | .40/.60    | 1.00/2.00  | .15/.25    | .002/.005 |

As representative of the properties of steel within these limits, as compared to prior art steel of the character aforesaid, I submit the data below:

of 12,000 pounds. These were .325 in. for steel D; .305 for steel K; .295 for steel E; and .265 for steel L.

To establish the relative hardenabilities of these

Table II

| Heat | Steel | Per Cent C | Per Cent Mn | Per Cent Si | Per Cent Ni | Per Cent Cr | Per Cent Mo | Per Cent B | Bal. |
|------|-------|------------|-------------|-------------|-------------|-------------|-------------|------------|------|
| 8983 | D     | .03        | .10         | .03         |             |             |             |            | Fe   |
| 8680 | E     | .05        | .36         | .20         | 1.21        | .61         |             |            | Fe   |
| 8676 | F     | .07        | .29         | .13         | .02         | .81         | .23         |            | Fe   |
| 8677 | G     | .07        | .35         | .14         | .03         | 1.19        | .23         |            | Fe   |
| 8678 | H     | .06        | .35         | .14         | .54         | 1.22        | .24         |            | Fe   |
| 8679 | J     | .06        | .37         | .19         | .56         | 1.30        | .25         | 0.0035     | Fe   |
| 8969 | K     | .07        | .37         | .20         | .50         | 1.47        | .22         | 0.0045     | Fe   |
| 8681 | L     | .06        | .38         | .23         | 3.51        | 1.47        |             |            | Fe   |

Of these, steel D is similar to steel A of Table I; steel E is similar to steel B; and steel L is similar to steel C. All the other steels are within the limits of this invention.

As fully annealed, the Brinell hardness values

steels, samples were tested by the conventional Jominy end-quench procedure, for both 1500F, and 1650F, austenitizing temperatures. The hardness values attained at the 2, 6, and 10 sixteenth positions on the test pieces are as follows:

Table IV

| Steel | Designation               | Rockwell "B" Hardness |      |        |      |         |      |
|-------|---------------------------|-----------------------|------|--------|------|---------|------|
|       |                           | Pos. 2                |      | Pos. 6 |      | Pos. 10 |      |
|       |                           | *1500                 | 1650 | *1500  | 1650 | *1500   | 1650 |
| L     | Higher Ni-Cr (per C)..... |                       |      | 108    | 105  | 103     |      |
| J     | This invention.....       | 94                    | 102  | 85.5   | 94   | 80.5    | 89   |
| H     | do.....                   | 92.5                  | 101  | 84     | 91.5 | 78      | 85.5 |
| G     | do.....                   | 89.5                  | 101  | 83     | 91   | 77      | 83.5 |
| F     | do.....                   |                       |      | 99     | 87   | 78.5    |      |
| E     | Lower Ni-Cr (per A).....  | 87                    | 97   | 76     | 83.5 | 72      | 77.5 |

\*Austenitizing temperature, ° F.

of these steels, and it may be taken that the hubbability varies inversely as the Brinell hardness, are as follows:

Further data on relative hardenabilities were obtained by testing the hardness and tensile properties of some of these steels as quenched in

1" round bars and tempered at 350F with results as follows:

Table V

| Steel | Designation    | Treatment        | Hardness<br>Brinell | Y. S.,<br>P. s. i. | T. S.,<br>P. s. i. | EI.,<br>Per Cent | R. A.,<br>Per Cent |
|-------|----------------|------------------|---------------------|--------------------|--------------------|------------------|--------------------|
| A     | Plain Carbon   | 1450F, water qu. | 120                 | 40,000             | 60,000             | 30               | 65                 |
| B     | Lower Ni-Cr    | 1500F, oil qu.   | 160                 | 50,000             | 80,000             | 30               | 65                 |
| K     | This invention | 1550F, oil qu.   | 160                 | 45,000             | 81,000             | 26               | 62                 |

Thus it has been shown that the steel of the present invention has a better combination of hubbability and hardenability than commercial steels heretofore known.

In the appended claims, by the expression "balance substantially all iron" is meant iron except for impurities within commercial tolerances.

I claim:

1. An alloy steel characterized by good hubbability and hardenability, containing about: 0.02 to 0.07% carbon; 0.3 to 0.5% manganese; 0.02 to 0.2% silicon; 0.4 to 0.6% nickel; 1 to 2% chromium; 0.15 to 0.25% molybdenum; 0.002 to 0.005% boron; and the balance substantially all iron.

2. A hubbed, carburized and heat treated mold die for molding resinous plastics, made of an alloy steel containing about, 0.02 to 0.15% carbon; 0.1 to 1.0% manganese; 0.8 to 3.0% chromium; 0.1 to 1.0% molybdenum; up to about 0.4% silicon; up to about 1.0% nickel; up to about 0.005% boron; and the balance substantially all iron.

3. A hubbed, carburized and heat treated mold die for molding resinous plastics, made of an alloy steel containing about: 0.02 to 0.07% carbon; 0.3 to 0.5% manganese; 0.02 to 0.2% silicon; 0.4 to 0.6% nickel; 1 to 2% chromium; 0.15 to 0.25% molybdenum; 0.002 to 0.005% boron; and the balance substantially all iron.

4. An alloy steel characterized by good hubbability and hardenability containing about: 0.02

to 0.15% carbon; 0.1 to 1.0% manganese; 0.8 to 3.0% chromium; 0.1 to 1.0% molybdenum; from an effective amount up to about 1% nickel; up to 15 about 0.4% silicon; up to about 0.005% boron; and the balance substantially all iron.

5. A hubbed, carburized and heat treated mold die, made of an alloy steel containing about: 0.02 to 0.15% carbon; 0.1 to 1.0% manganese; 0.8 to 3.0% chromium; 0.1 to 1.0% molybdenum; from an effective amount up to about 1% nickel; up to about 0.4% silicon; up to about 0.005% boron; and the balance substantially all iron.

PETER PAYSON.

25

#### REFERENCES CITED

The following references are of record in the file of this patent:

#### UNITED STATES PATENTS

| Number    | Name        | Date          |
|-----------|-------------|---------------|
| 1,519,383 | Walter      | Dec. 16, 1924 |
| 2,283,299 | Tisdale     | May 19, 1942  |
| 2,332,441 | Fleischmann | Oct. 19, 1943 |

30

#### OTHER REFERENCES

Chemical Engineers Handbook, second edition, page 2113, Alloy No. 91. John H. Perry, editor. Published in 1941 by the McGraw-Hill Book Company, New York.

35

40